

## UNITED STATES PATENT OFFICE.

DANIEL H. MELOCHE, OF DETROIT, MICHIGAN, ASSIGNOR TO EARL HOLLEY, OF DETROIT, MICHIGAN.

## METHOD OF PRODUCING GRAY-IRON CASTINGS.

No Drawing. Application filed January 31, 1924, Serial No. 689,816. Renewed November 30, 1925.

This invention relates to the method of producing gray iron castings of a superior quality.

When gray iron is cast in sand molds a characteristic structure is produced in which large crystals of graphite exists in a matrix of ferrite. This iron is soft, easily machinable, and of good wearing qualities. Millions of tons of this iron are cast every year.

This iron, however, exhibits strength in neither compression nor tension and is easily broken by impact. There is a demand therefore for an iron having all the good qualities of gray iron, together with greater strength and resistance to impact.

When iron is cast in a heated metal mold protected with a refractory lining and a superimposed coating of lampblack, as described in my co-pending application Serial No. 623,053, allowed October 17th, 1923, the iron produced thereby has the good qualities of gray iron but is not markedly superior to gray iron in strength and resistance to impact.

I have discovered, however, that if I anneal such an iron at 1550° F. for one hour, that whilst the characteristic structure of such iron is unchanged the strength is increased 100%. On the other hand, if the annealing is continued at this temperature for two or three hours the characteristic structure is destroyed and the iron is weaker than ordinary sand cast iron.

The explanation of this remarkable increase in strength is believed to be as follows:—

When gray iron, containing over 2.2% silicon and over 2.5% carbon (preferably 2.75% silicon, 3.25% carbon, and 0.6% manganese), is cast in heated metal molds, protected as described above, whilst the initial rate of cooling is checked the average rate of cooling is greater than when using sand

molds, the result being that the silicon precipitates out the carbon as minute particles of graphite entirely surrounded by ferrite.

The specific gravity of graphite being but 30% of the specific gravity of pure iron (ferrite) the volume of the mass increases at the moment of precipitation, the result being that each particle of graphite is surrounded by an envelope of ferrite in tension and there are therefore casting strains uniformly distributed throughout the iron, and it is to relieve these casting strains that the short anneal of one hour at 1550° is used rather than a longer anneal.

It will be noted that this anneal is not intended to change either the chemical composition or physical appearance of the casting. However, the anneal actually does cause some of the combined carbon that has escaped the effect of the silicon to come out of solution. This is not intended however. Generally speaking, there is no material change in the structure.

What I claim is:

1. The method of making gray iron castings consisting of casting such iron in a heated metal mold protected with a heat insulating refractory and a superimposed coating of lampblack, removing the casting from said mold and heating the casting above 1475° F. and below 1600° F. long enough to relieve the casting strains and not long enough to destroy the characteristic structure of the iron.

2. A gray iron casting containing more than 2.2% silicon and more than 2.5% carbon, characterized by the uniform distribution of 90% of the carbon as particles of graphite surrounded by ferrite, annealed so as to relieve the casting strains and so as not to materially change the characteristic structure of the metal.

In testimony whereof I affix my signature.

DANIEL H. MELOCHE.